

## UNITED STATES PATENT OFFICE

WERNER BUSCH, OF COLOGNE-DEUTZ, AND ERICH NOACK, OF WIESDORF, GERMANY,  
ASSIGNORS TO I. G. FARBBENINDUSTRIE AKTIENGESELLSCHAFT, OF FRANKFORT-  
ON-THE-MAIN, GERMANY, A CORPORATION OF GERMANY

## MANUFACTURE OF POTASSIUM

No Drawing. Application filed July 21, 1928, Serial No. 294,576, and in Germany August 5, 1927.

This invention relates to the manufacture of potassium.

The process of manufacture in accordance 5 with this invention is by heating potassium fluoride with metallic magnesium in the absence of water. This process offers quite considerable technical advantages since the reaction commences at a temperature above 10 about 500° C. and is complete at a low red heat, taking place smoothly and with a good yield. Advantageously the process is carried out in an inert atmosphere or better still under reduced pressure. Iron is an example 15 of a suitable material for the reaction vessels. The potassium obtained in this manner is very pure. The residue from the reaction can be worked up in the known manner to give pure magnesium fluoride or 20 hydrofluoric acid and magnesium salts.

The following example illustrates the invention without limiting it thereto:—

A mixture of 90 grams of thoroughly 25 dessicated potassium fluoride and 18 grams of magnesium grit is heated to about 500-700° C. in an iron retort under about 11 mm. pressure. When a temperature of 540° C. is reached, the potassium distils over and is 30 collected in the form of balls in a receiver charged with a suitable liquid inert towards potassium, such as petroleum, paraffin oil e. a. The yield of potassium amounts to 48 grams, it contains only barely detectable 35 traces of magnesium.

We claim:—

1. In the process of manufacturing potassium the step which comprises heating potassium fluoride with metallic magnesium to a temperature above about 500° C. in the absence of water and under reduced pressure.
2. A process of manufacturing potassium 45 which process comprises heating thoroughly

dried potassium fluoride with magnesium to about 500-700° C. under about 11 mm. pressure and collecting the potassium distilling over in a receiver charged with a suitable 50 liquid inert towards potassium.

In testimony whereof we have hereunto set our hands.

WERNER BUSCH. [L. S.]

ERICH NOACK. [L. S.]

55

60

65

70

75

80

85

90